

Sept. 13, 1960

A. ARMEN ET AL  
FORMATION WITH CERTAIN ALCOHOLS OF ACRYLAMIDE GROUPS  
ON POLYACRYLONITRILE IN ZINC CHLORIDE SOLUTION  
Filed May 7, 1958

2,952,651

Amide Formation vs Time for *t*-Butyl Alcohol  
and Polyacrylonitrile-Polyacrylonitrile  
Dissolved in 60% Aqueous  $ZnCl_2$



INVENTORS.

Ardy Armen  
BY Stanley A. Murdock

*Jerome Rudey*

ATTORNEY

1

2,952,651

FORMATION WITH CERTAIN ALCOHOLS OF  
ACRYLAMIDE GROUPS ON POLYACRYLONITRILE IN ZINC CHLORIDE SOLUTIONArdy Armen and Stanley A. Murdock, Concord, Calif.,  
assignors to The Dow Chemical Company, Midland,  
Mich., a corporation of Delaware

Filed May 7, 1958, Ser. No. 733,624

10 Claims. (Cl. 260—29.6)

The chief aim and major concern of the present invention is to provide an improved process for modifying polyacrylonitrile of the fiber-forming variety so as to enhance its dye-receptivity while the polymer is dissolved in an aqueous, zinc chloride-containing solvent therefor as a spinnable composition that is adapted to be wet-spun (by salt-spinning procedures according to the conventional technique) into readily dyeable filamentary and the like shaped articles and products.

To this end, dye-receptive alkyl acrylamide groups or units may be introduced into fiber-forming polyacrylonitrile while it is in the form of a wet spinnable, fiber-forming solution in an aqueous, polyacrylonitrile-dissolving solvent comprised of zinc chloride by a method which, surprisingly and simply enough, comprises adding to the polymer-containing aqueous saline spinning solution a minor proportion of tertiary alcohol or a benzyl alcohol, or a mixture thereof, as hereinafter defined, and heating the mixture at a temperature between about 50° C., preferably at least about 60° C. and 80° C. or so for a period of time between about 0.1 and 25 hours until between about 2 and 25 mole percent of the nitrile groups preferably between about 8 and 20 mole percent thereof, are converted to alkyl acrylamide units corresponding to the substituents introduced by the particular alcoholic reactant (or mixture of reactants) employed. The resulting acrylonitrile polymer composition is especially well adapted to be salt-spun into excellent quality acrylonitrile polymer synthetic textile fiber products, using the well known wet spinning process in which aquagel intermediates are formed. The resulting fiber products which are obtained after irreversible drying of the aquagel intermediate that is coagulated from the modified spinning composition have excellent receptivity of and unusual affinity for dyestuffs of the acid class.

The tertiary and benzyl alcohols which may be utilized in the practice of the present invention to modify the fiber-forming polyacrylonitrile while it is dissolved in the zinc chloride-containing aqueous saline solvent therefor are any of those of the respective formulae:



wherein each R is independently a 1 to about 4 carbon atom-containing alkyl unit with the limitation that the total number of carbon atoms in all three R substituents is from 3 to 7; and



wherein each X is independently selected from the group consisting of halogens of atomic number 17 to 35 (i.e., chlorine and bromine), and alkyl radicals containing from 1 to about 4 carbon atoms; and n has a whole number value from 0 to 5. Advantageously, the dis-

2

solved polyacrylonitrile is modified with tertiary-amyl alcohol ( $C_2H_5(CH_3)_2COH$ ), tertiary-butyl alcohol ( $((CH_3)_3COH$ )

5 benzyl alcohol, or mixtures thereof. Excellent results may also be obtained, however, by use of such alcohols as 3-methyl-pentane-3-ol ( $((C_2H_5)_2CH_3COH$ ), 2-methylpentane - 2 - ol ( $C_3H_7(CH_3)_2COH$ ), 3-ethyl-pentane-3-ol ( $((C_2H_5)_3COH$ ), 3-methyl-hexane-3-ol



2-methyl-hexane-2-ol ( $C_4H_9(CH_3)_2COH$ ), p-chloro-benzyl alcohol, 2,4-dibromo-benzyl alcohol, 2-chloro-4-methyl-benzyl alcohol and others of those within the scope of

15 the Formulae I and II as well as various mixtures of any or all of such species.

The reaction of the alcohol with the polyacrylonitrile while the latter is dissolved in spinnable concentration in the aqueous, polyacrylonitrile-dissolving, zinc chloride-containing solvent therefor modifies the polymer, by means other than copolymerization, to obtain a resulting fiber-forming acrylonitrile polymer product which, in effect, is essentially a copolymer, containing intermixtures of recurring acrylonitrile and alkyl acrylamide units

25 in the polymer molecule, as typified by the following:



30 wherein the value of z is from 2 to 25 mole percent, preferably from 8 to 20 mole percent, of the sum of y plus z, and the G substituent, depends upon the particular alcohol (or alcoholic mixture) used for the modification of the polyacrylonitrile.

35 This modification occurs by the following reactions: with tertiary alcohols of Formula I



with benzyl alcohols of Formula II



55 The precise quantity of the alcohol that is utilized depends upon the degree of modification of the polyacrylonitrile that is desired (i.e., the proportion of recurring alkyl acrylamide units desired to be introduced therein), the extent towards completion which the reaction is permitted to proceed, and the particular alcohol utilized. In any event, the quantity to employ in any given situation can be readily calculated, taking the above factors into account. In many cases, without intending to be limited thereto, satisfactory results can be achieved 60 when between about 2 and 25 mole percent, advantageously about 10 mole percent, of the alcohol is employed, based on the molar quantity of polyacrylonitrile being modified in the spinning solution.

70 The aqueous salt solution comprising zinc chloride which is employed as the solvent for the polyacrylonitrile in the practice of the invention is preferably a 55 to 65 percent by weight solution, preferably about a 60 weight

percent solution, of zinc chloride as the sole saline constituent.

The amount of polyacrylonitrile that is modified in the aqueous saline spinning solution may advantageously be between about 2 and 20 percent by weight, based on the weight of the polymer-containing spinning solution. More often, it may be more beneficial for the spinning solution to contain between about 6 and 15 weight percent, and even more beneficially from 8.5 to 11.5 weight percent, of dissolved polymer. Generally, it is preferable for the polyacrylonitrile that is modified to be in the desirable molecular weight range from about 20,000 to 60,000 (viscosimetrically determined as described in United States Letters Patent No. 2,763,636, at column 2, lines 37-41) and the solution itself in the viscosity range, measured at about 35° C., of from about 300 to 3,000 poises. Of course, lower and higher molecular weight polyacrylonitrile can also be modified to enhance its dye-receptivity by practice of the invention. The modified spinning solutions of the present invention can be salt-spun in the known manner to form synthetic textile fiber products, or films if desired, using non-polyacrylonitrile-dissolving aqueous solutions of zinc chloride as the coagulating spin bath for the extruded products. Thus, the aqueous coagulating baths in which the aquagel structures are formed may advantageously contain between about 25 and 50 weight percent of dissolved salt, more advantageously from about 30 to 45 weight percent, and preferably in the neighborhood of 42-43 weight percent.

In conducting the alcohol modification of the dissolved polyacrylonitrile to introduce alkyl acrylamide units therein, care should be taken to avoid use of too high a temperature for too long a period of time in order to circumvent the possibility of hydrolyzing the acrylonitrile polymer in solution. Thus, when temperatures of about 95° C. are employed, it is generally found that appreciable hydrolysis results. This, of course, causes highly undesirable consequences in the procedure.

By way of further illustration, a series of polyacrylonitrile spinning solution samples were prepared containing about 10 weight percent of dissolved polyacrylonitrile having an average molecular weight of about 28,000 in 60 percent by weight aqueous zinc chloride solution. The polymer was prepared by direct solution polymerization of monomeric acrylonitrile in the aqueous saline solvent. Prior to polymerization, the aqueous zinc chloride solution had been adjusted to pH 3 (measured at 10:1 by volume aqueous dilution) with hydrochloric acid. Into each of the samples was added about 10 weight percent of tertiary-butyl alcohol, based on the weight of the dissolved polymer in the spinning solution. The alcoholic reactant was added to each sample as an equal weight mixture with 60 percent aqueous zinc chloride to prevent coagulation of the polymer solution. Addition of the alcohol was made to each sample after it had been heated to the desired temperature of reaction at which it was maintained during the experimentation. Reaction temperatures of 40° C., 60° C., 80° C., and 95° C. were used. All of the samples were stirred throughout their modification. In order to check hydrolysis, a non-alcoholic blank was run at 40° C. At reaction temperatures up to about 80° C., the degree of hydrolysis incurred by the modification was relatively insignificant. Hydrolysis became appreciable and occurred to an undesirable extent at 95° C. The results are set forth in the sole figure of the accompanying drawing, wherein the essential data from the several samples at various reaction temperatures are graphically portrayed by plotting reaction time against relative amide formation in the modified polyacrylonitrile, expressed as mole percent of alkyl acrylamide units found in the resulting polymer samples by means of infrared analysis.

By way of still further illustration, a modified spinning solution was prepared in the foregoing manner to obtain an acrylonitrile polymer in 60 percent aqueous zinc

chloride spinning solution containing about 10 percent by weight of dissolved polymer solids consisting of polyacrylonitrile modified with tertiary-butyl alcohol for 10 hours at 60° C. until about 14 mole percent of alkyl acrylamide units were introduced in the fiber-forming polymer. The spinning solution was extruded into an aqueous coagulating bath therefor containing about 43 weight percent of dissolved zinc chloride. A 750 hole spinnerette was employed in which each orifice had an individual diameter of about 6 mils. After extrusion, the aquagel fibers were wet-stretched about twelve times for orientation, washed thoroughly with water, then irreversibly dried for 30 minutes at 150° C. to synthetic acrylonitrile polymer fibers of about 3 denier/filament.

15 The fiber product had excellent physical characteristics, being about commensurate in its essential textile properties to ordinary polyacrylonitrile fibers. In addition, the modified fibers were found to be readily dyeable to level shades of coloration with Calcocid Alizarine Violet, an acid dye (Colour Index 1080); and many other acid dyestuffs of practical and commercial interest.

Excellent results similar to those demonstrated in the foregoing can also be obtained when the acrylonitrile is modified with tertiary-amyl alcohol, benzyl alcohol, or 25 any other of the alcoholic reagents or their mixtures read upon by the Formulae I and II. Excellent results are also obtained when other degrees of modification of the polyacrylonitrile in addition to those specifically illustrated are effected by the modifying treatment of the 30 present process.

What is claimed is:

1. Method for improving the dye-receptivity of fiber-forming polyacrylonitrile while it is dissolved as a spinable solution in an amount between about 2 and 20 weight percent, based on the weight of said solution, in an aqueous, polyacrylonitrile-dissolving, saline solution that is comprised of at least about 55 weight percent, based on the weight of the aqueous solution, of zinc chloride as the essential saline constituent, which method 35 comprises adding to said solution of polyacrylonitrile at least one alcohol selected from the group of those consisting of the formulae:



45 in which each R is an independent alkyl radical containing from 1 to about 4 carbon atoms with the limitation that the total number of carbon atoms in all of the R substituents of said alcohol of the Formula I is from 3 to 7; and



50 in which each X is independently selected from the group consisting of halogens of atomic number 17 to 35 and alkyl radicals containing from 1 to about 4 carbon atoms, and n has a whole number value from 0 to 5; and mixtures of alcohols of the Formulae I and II, said alcohol being added to said polyacrylonitrile solution in 55 an amount that is sufficient, upon subsequent reaction, to convert between about 2 and 25 mole percent of the nitrile groups in said polyacrylonitrile to alkyl acrylamide units; then heating the mixture of said alcohol and said solution of polyacrylonitrile at a temperature between about 40° C. and about 80° C. for a period of time between about 0.1 and 25 hours until between about 60 2 and 25 mole percent of the nitrile groups of said polyacrylonitrile are converted to dye-receptive alkyl acrylamide groups corresponding to the alcoholic reagent utilized for the modification.

65 2. The method of claim 1, wherein the amount of alcohol employed is an amount that is sufficient to convert between about 8 and 20 mole percent of said nitrile groups in said polyacrylonitrile to said alkyl acrylamide units.

3. The method of claim 1, wherein between about 2 and 25 mole percent, based on the molar quantity of polyacrylonitrile in solution, of said alcohol is added to said solution of said polyacrylonitrile.

4. The method of claim 1, wherein said spinnable composition of polyacrylonitrile contains between about 6 and 15 weight percent, based on the weight of the solution, of polyacrylonitrile dissolved in said aqueous, polyacrylonitrile-dissolving, saline solution and wherein about 10 mole percent, based on the molar quantity of polyacrylonitrile in solution, of said alcohol is added to said solution of polyacrylonitrile.

5. The method of claim 1, wherein said aqueous, polyacrylonitrile-dissolving, saline solution consists of between about 55 and 65 weight percent of zinc chloride in water, based on the weight of the aqueous solution.

6. The method of claim 1, wherein said mixture of alcohol and said solution of polyacrylonitrile is heated at a temperature between about 60° C. and about 80° C.

7. The method of claim 1, wherein said alcohol is tertiary-butyl alcohol.

8. The method of claim 1, wherein said alcohol is tertiary-amyl alcohol.

5 9. The method of claim 1, wherein said alcohol is benzyl alcohol.

10 10. The method of claim 1 and including, in addition thereto and in combination therewith, the step of extruding said resulting spinnable solution of the modified polyacrylonitrile after termination of said reaction with alcohol into an aqueous coagulating bath therefor to form coagulated shaped articles of said modified polyacrylonitrile in said bath.

15 References Cited in the file of this patent

UNITED STATES PATENTS

|           |                |       |                |
|-----------|----------------|-------|----------------|
| 2,648,647 | Stanton et al. | ----- | Aug. 11, 1953  |
| 2,719,144 | Shearer et al. | ----- | Sept. 27, 1955 |
| 2,847,389 | Evans          | ----- | Aug. 12, 1958  |